

UNITED STATES PATENT OFFICE

2,588,538

## STABILIZERS IN PHOTOGRAPHIC EMULSIONS AND DEVELOPERS

**John David Kendall and Harold Gordon Suggate,  
Ilford, England, assignors to Ilford Limited,  
Ilford, England, a British company**

**No Drawing. Application August 3, 1949, Serial  
No. 108,418. In Great Britain August 6, 1948**

**15 Claims. (Cl. 95—7)**

1

This invention relates to compounds which serve as "anti-fogging agents" or "stabilizers" for photographic silver halide emulsions and which may be used as additions to the emulsions or to the developers used in processing emulsions.

On exposure and development of a normal photographic film, plate or paper bearing a silver halide photographic emulsion there is produced, in addition to the silver image, a general deposit of metallic silver, the distribution and density of which bears no relation to the variations in luminosity of the subject. This overall deposit is referred to as the "chemical fog" or "development fog." Its effect is to increase the general density of the negative obtained and to depress the contrast of the image in the less exposed parts. In general the fog density produced is greater in the case of high speed than in slow emulsions and is invariably greater the higher the temperature of development and when vigorous developers are used. Moreover, the degree to which an emulsion produces fog on development usually increases with the age of the emulsion so that photographic materials which have been kept a long time, especially in warm and humid conditions, or emulsions which have been kept a long time in the molten condition, may produce images associated with a heavy fog density. Many compounds have been suggested in the past for use as additions to emulsions or to developers which tend to reduce the formation of fog, but almost all of them, if reasonably effective as anti-fogging agents, have caused a serious reduction in the speed of the photographic emulsion.

According to the present invention the tendency to the formation of fog in silver halide photographic emulsions is reduced by incorporating in the emulsion or the developer or both a small quantity of a compound of the general formula:



(or a tautomer thereof) where  $R_1$  is a hydrogen atom or an alkyl group.

It has been found that such compounds are very effective anti-fogging agents both in developers and in emulsions. They preserve high speed emulsions against excessive fog over long periods of time and they enable development to be effected with vigorous developers or at high temperatures. Thus the compounds are of particular value as emulsion or developer additions.

2

in cases where the emulsions or developers are to be used in tropical conditions or, in the case of emulsions, where the emulsions are to be kept for a long time in the molten condition.

5 The compounds present the further advantage that they do not seriously reduce the effective speed of emulsions in which they are incorporated.

10 The new anti-fogging agents may be prepared by the processes described in our co-pending application Serial No. 108,417, now U. S. Patent No. 2,534,914, filed on even date herewith.

As indicated above the group  $R_1$  in the general formula may be a hydrogen atom or an alkyl group. Examples of suitable alkyl groups are methyl, ethyl and higher alkyl groups.

The quantity of the compound employed will depend on the emulsion or the developer to which it is added, but as a general indication it may be stated that for incorporation in an emulsion, 1 to 5 or up to 50 cc. of a 1:1,000 solution of the compound per litre of emulsion is suitable, whilst for incorporation in a developer, the optimum quantity may vary from 1 part of the compound in 3,000 to 30,000 parts of the developer solution according to the particular compound used. The addition of the compound to an emulsion is preferably effected after the digestion of the emulsion as a final addition before coating.

The following examples illustrate the invention:

### Examples

35 To an iodobromide emulsion containing 1½ gram-molecules of silver were added 20 cc. of a 1:1000 ethyl alcohol solution of 3,3'-bis(1,2,4-triazolyl)-formamidine. The emulsion was then coated on glass, dried and stored, part of the product under normal conditions and part in a sealed container at 120° F. A control emulsion containing no stabiliser was similarly treated. Sensitometric results were as follows:

| 45 | Compound                                                    | Normal keeping |                    | Keeping 8 days at 120° F. |                              |
|----|-------------------------------------------------------------|----------------|--------------------|---------------------------|------------------------------|
|    |                                                             | Fog            | Relative log speed | Fog                       | Relative log speed (inverse) |
| 50 | (Control)<br>3,3'-bis(1,2,4-triazolyl)-<br>formamidine----- | 0.06           | 3.70               | 0.28                      | 3.65                         |
|    |                                                             | 0.06           | 3.69               | 0.11                      | 3.85                         |

It will be seen that the emulsion containing the stabiliser gave less fog than the control on keeping, but without serious effect on the speed

of the emulsion which was lowered only slightly. Similar results were obtained using—

3.3'-bis(5-methyl-1.2.4-triazolyl)-formamidine  
3.3'-bis(5-ethyl-1.2.4-triazolyl)-formamidine

What we claim is:

1. A process for reducing the tendency to the formation of fog in silver halide photographic emulsions which comprises developing the emulsions, in the presence of a small quantity of a compound of the general formula:



where  $R_1$  is selected from the class consisting of the hydrogen atom and alkyl groups.

2. A process for reducing the tendency to the formation of fog in silver halide photographic emulsions which comprises developing latent images in such emulsions by means of a developing solution containing a small quantity of a compound of the general formula:



where  $R_1$  is selected from the class consisting of the hydrogen atom and alkyl groups.

3. A process for reducing the tendency to the formation of fog in silver halide photographic emulsions which comprises developing latent images in such emulsions by means of a developing solution containing a small quantity of a compound of the general formula:



where  $R_1$  is selected from the class consisting of the hydrogen atom and alkyl groups, the quantity of the said compound included in the developer being equivalent to 1 part of the compound per 3000 to 30,000 parts of the developing solution.

4. A process for reducing the tendency to the formation of fog in silver halide photographic emulsions which comprises developing the emulsions, in the presence of a small quantity of 3.3'-bis(1.2.4-triazolyl)-formamidine.

5. A process for reducing the tendency to the formation of fog in silver halide photographic emulsions which comprises developing the emulsions, in the presence of a small quantity of 3.3'-bis(5-methyl-1.2.4-triazolyl)-formamidine.

6. A process for reducing the tendency to the formation of fog in silver halide photographic emulsions which comprises developing the emulsions, in the presence of a small quantity of 3.3'-bis(5-ethyl-1.2.4-triazolyl)-formamidine.

7. A photographic silver halide emulsion containing a small quantity of a compound of the general formula:



where  $R_1$  is selected from the class consisting of the hydrogen atom and alkyl groups.

8. A photographic silver halide emulsion containing in the proportion of 1 to 50 cc. of a 1:1000 solution per litre of emulsion a compound of the general formula:



where  $R_1$  is selected from the class consisting of the hydrogen atom and alkyl groups.

9. A photographic silver halide emulsion containing in the proportion of 1 to 50 cc. of a 1:1000 solution per litre of emulsion 3.3'-bis(1.2.4-triazolyl)-formamidine.

10. A photographic silver halide emulsion containing in the proportion of 1 to 50 cc. of a 1:1000 solution per litre of emulsion 3.3'-bis(5-methyl-1.2.4-triazolyl)-formamidine.

11. A photographic silver halide emulsion containing in the proportion of 1 to 50 cc. of a 1:1000 solution per litre of emulsion 3.3'-bis(5-ethyl-1.2.4-triazolyl)-formamidine.

12. A photographic developing composition including a silver halide photographic developer and a small quantity of a compound of the general formula:



where  $R_1$  is selected from the class consisting of the hydrogen atom and alkyl groups.

13. A photographic developing solution containing a silver halide photographic developer and, per 3000 to 30,000 parts of the solution, 1 part of 3.3'-bis(1.2.4-triazolyl)-formamidine.

14. A photographic developing solution containing a silver halide photographic developer and, per 3000 to 30,000 parts of the solution, 1 part of 3.3'-bis(5-methyl-1.2.4-triazolyl)-formamidine.

15. A photographic developing solution containing a silver halide photographic developer and, per 3000 to 30,000 parts of the solution, 1 part of 3.3'-bis(5-ethyl-1.2.4-triazolyl)-formamidine.

JOHN DAVID KENDALL.  
HAROLD GORDON SUGGATE.

#### REFERENCES CITED

The following references are of record in the file of this patent:

#### UNITED STATES PATENTS

| Number    | Name     | Date          |
|-----------|----------|---------------|
| 1,763,989 | Sheppard | June 17, 1930 |
| 2,153,930 | Kendall  | Apr. 11, 1939 |
| 2,353,754 | Peterson | July 18, 1944 |
| 2,475,136 | Heimbach | July 5, 1949  |
| 2,476,525 | Anish    | July 19, 1949 |
| 2,534,914 | Kendall  | Dec. 19, 1950 |